

March 3, 1931.

R. E. DRAKE

1,794,449

BUILDING PRODUCT AND PROCESS FOR MAKING THE SAME

Filed Oct. 8, 1926

Fig.1.



Fig. 2.



Fig. 3.



Fig. 4.



Fig. 5.



INVENTOR  
Ralph E. Drake  
BY  
Lennie, Davis, Marion Edwards  
ATTORNEYS

## UNITED STATES PATENT OFFICE

RALPH E. DRAKE, OF JAMAICA, NEW YORK, ASSIGNOR, BY MESNE ASSIGNMENTS, TO  
ANACONDA SALES COMPANY, OF NEW YORK, N. Y., A CORPORATION OF DELAWARE

## BUILDING PRODUCT AND PROCESS FOR MAKING THE SAME

Application filed October 8, 1926. Serial No. 140,247.

This invention relates to the manufacture of composite building elements suitable for roofing and other purposes and comprising a non-metallic base material and a sheathing of 5 weather-resistant metal applied to the surface thereof. More particularly, the invention relates to an electrolytic process for the application of metal to bases of this type in the manufacture of such composite products. 10 This process is of primary utility in the application of copper, which is the metal principally used in building elements of this kind, owing to the resistance which copper offers to corrosion, and its attractive appearance, but 15 the utility of the invention is by no means limited to the application of copper, nor to the use of any specific base material.

Owing to the high cost of wooden shingles, and their low fire resistance, numerous prepared roofings are now in extensive use, these 20 products being made of roofing felt, asbestos board, magnesite compositions and the like. The felt product now enjoys the widest popularity and it is made of a felt of suitable 25 weight and thickness which is ordinarily saturated with bituminous products, such as asphalt, and then coated with a layer of asphalt which is capable of withstanding solar heat. Sometimes the felt has an additional 30 coating of granular material such as crushed slate, which improves its wearing qualities and increases its resistance to fire. Roofing products of this kind are in general satisfactory but their appearance on the roof is somewhat monotonous and when not properly 35 made, the edges of the overlapping elements have a tendency in time to warp and curl, making the roof unsightly and possibly subject to leakage.

40 It has been proposed heretofore to use materials of this type in a composite product which includes an additional layer of metal applied to that area of the element which is exposed to the weather. A layer of copper thus applied gives the roof the appearance of 45 being covered with copper sheathing and such a roof is of handsome appearance, and of high fire resistance and long life. The difficulty involved in making such a roofing is to secure 50 a good bond between the base and metal, for

the two expand and contract at different rates and exposure to the weather is likely to cause the metal sheathing to come loose from the base.

One proposal in an effort to overcome this 55 suggests the application of the metal to a base which has a rough and irregular surface due to the application of a layer of granular material, such as crushed slate. The slate may be embedded partially in the asphalt coating 60 layer on the base and the slate granules which are of substantial size project beyond the base and form crests and depressions. When the metal is applied electrolytically over such a 65 surface, the metal enters the depressions and conforms to the irregularities of the surface, so that a firm mechanical bond is established. In addition, the different parts of the metal sheet expand and contract in different planes 70 so that the expansion effect is not cumulative throughout the sheet in a horizontal plane.

While the grit surfaced base coated with 75 metal is thus far superior to a plain surfaced product, attempts to apply the metal electrolytically have met with numerous obstacles. An electroconductive material must be applied to the base in order to permit the electrodeposition of the metal and graphite, which is the simplest and cheapest material to use, can be applied in a thin continuous 80 film over all parts of the irregular base surface only with considerable difficulty, and by the use of an adhesive. Any failure to produce a film which enters all the depressions and extends over all the crests results in an 85 imperfect product and adds largely to the cost of production owing to the increased electrical resistance of the film.

This difficulty has been overcome by substituting for the granular material ordinarily used for roofing purposes, an electroconductive material of granular form, as distinguished from the electroconductive powder or graphite ordinarily used. This material may be crushed petroleum coke, or the like, 95 and the individual pieces are about the same size as the particles of slate ordinarily used. The electroconductive material is affixed to the base by being partially embedded in the 100 coating layer of asphalt over the felt in the

usual way, and since the granules are of considerable size and are conductive, they provide the irregular surface on the base and also the conductive surface needed for the 5 electrodeposition.

In the use of the electroconductive granular material above mentioned I have found that the granules of the irregular layer must be in close contact throughout the surface of 10 the base in order that a substantially continuous conductive surface may be provided on which the metal is deposited, and any failure in this respect results in the production of a plating which has gaps and also the cost of 15 the operation is high because of the low conductivity of the discontinuous cathode surface.

It is the object of this invention to provide a process of producing building elements of the composite type electrolytically 20 which may be carried on more easily than those heretofore employed and which produces better results because the process yields a higher percentage of perfect elements. 25 This process involves the application of an electroconductive granular material to the surface of the base so that the latter has the desired conductive surface and the irregular contour, but this granular material is selected and graded so that a layer of it applied to the base is substantially continuous 30 with respect to its conductivity. This result is obtained by preparing a granular material in which the granules are of different sizes, 35 selected so that in a mass of granules the voids are considerably less than those present in an ungraded grit. When such a material is applied to the surface of the base in the usual way, a layer results in which each particle 40 is in close contact with those adjacent, due to the intermixture of large and small granules, the smaller granules filling the spaces between the larger ones and insuring this contact, while the large granules project from 45 the base and produce the irregularity desired. The metal is plated over this granular surface in the usual way.

Instead of using a graded grit made of 50 granules of different sizes in suitable proportions, I may secure the desired continuity in the conductive film by using an ungraded grit of particles of different sizes just as it comes from the crushers, where the grit 55 masses have been reduced to particles of a given maximum size suitable in a product of this type. But when such a grit is employed, I first embed the grit and then apply a thin film of graphite. The graphite may 60 be brushed on or applied in any convenient manner, and no considerable care in its application is required. The graphite thus applied finds lodgment in the crevices between the grit particles, covers any asphalt exposed 65 between adjacent particles and some of the

graphite adheres to the exposed surfaces of the grit to provide with the grit a continuous electroconductive layer. When ordinary grit and an adhesive are used, the graphite or other conductor must be spread with extreme care and it is almost impossible to 70 make it adhere to the projecting points of the granules, but in the new process, this extreme care is not necessary for the graphite is intended only to bridge the spaces between the adjacent conductive particles and lodges 75 readily between them. Accordingly, the graphite which acts chiefly to augment the conductivity of the granular layer, may be applied with great rapidity and by an attendant of only ordinary skill.

The invention includes not only a process of producing building products of the composite type but also the improved product resulting from the use of this process. This 80 product has important advantages over those previously produced in that a firm bond between base and metal is secured, the metal layer is continuous throughout, and the product may be made more cheaply, owing to the 85 lower number of imperfect elements in a given run.

For a better understanding of the invention, reference may be had to the accompanying drawing, in which,

Fig. 1 is a plan view of a rectangular building element made in accordance with the invention, the layer of material on the base being broken away for purposes of illustration,

Fig. 2 is a vertical sectional view on an enlarged scale,

Fig. 3 is a view similar to Fig. 2, but with the granular material shown somewhat enlarged, this material being graded as to size,

Fig. 4 is a view similar to Fig. 3, with the granular material ungraded and with graphite or similar conductive powder also used,

Fig. 5 is a plan view of a portion of the granular layer ready to be plated.

Referring to the drawings, Fig. 1 shows a building element in approximately the shape of an ordinary shingle, the element comprising a base 10, a coating layer 11 thereon, a layer of granular material 12 applied to the surface of the coated base, and a layer 13 of metal forming the outer protective film over a part of the base.

The base 10 may be of any convenient material, such as asbestos board, paper and the like, but is preferably the usual roofing felt saturated with a waterproofing material, such as asphalt. The surface of this base has the coating 11 which may conveniently consist of an application of asphalt, preferably one having a higher melting point than that used as a saturant, and capable of withstanding solar heat without running. This

coating layer adds to the waterproof qualities of the base and also acts as an adhesive for the granular material 12, the latter being partially embedded in the coating by pressure before the coating has set.

The granular material which I prefer to employ is preferably of a carbonaceous character and I have found that calcined petroleum coke, metallurgical coke, coke obtained from coal tar pitch, and carbon obtained by the calcining of anthracite coal are satisfactory for the purpose. These materials possess the necessary electrical conductivity, are readily obtainable, and easily crushed.

I have found that the size of the particles of conducting material to be used to provide the cathode surface on the elements over which metal is to be plated is of importance for if the conductive material used is made up of particles which are very fine, it is difficult to produce a layer of such particles of uniform thickness, in which all the particles are in contact, unless excessive quantities of the material are used. Then, when the layer is subjected to pressure to cause the particles to be affixed, many of the particles become submerged and are thus quite useless. Unless contact is made between adjacent particles, so that the layer is continuous as to its conductivity, the metal plating is not continuous and it is not uniformly thick. Also, as the conductivity of a non-continuous layer is low, the cost for plating current becomes high. Also, if material made up of fine particles is used to the extent necessary to produce a continuous conductive film, some of the particles will not become firmly affixed to the base and thus the bond between the metal coating and the base will be weak.

If the particles employed are of too large a size so that an appreciable portion of each particle is submerged in the plastic coating on the base, there is a likelihood of lack of contact, although the bond between such metal as can be deposited, and the base, is quite good.

Accordingly, it will be seen the size of the granules has an important bearing on the excellence of the finished product and its manufacture, and I have found that best results are obtained when the granular material is made up of particles of predetermined sizes, so graded as to size and proportioned as to amounts as to produce a mixture of fine and coarse particles which may be applied in a thin layer on the face of a sheet in such manner that the finer particles largely fill the spaces between the coarse particles so that each particle contacts with those adjacent to it. By the use of such a mixture there are secured maximum contact and optimum conductivity in the granular layer.

In the grading of the granular material, I

have found that a material of the following composition is satisfactory:

|                              | Per cent |
|------------------------------|----------|
| Retained on a 14 mesh screen | 0        |
| Retained on a 20 mesh screen | 5        |
| Retained on a 35 mesh screen | 20       |
| Retained on a 48 mesh screen | 50       |
| Retained on a 65 mesh screen | 25       |

This material is substantially free from dust, which would interfere greatly with its application and also with the adherence of the mixture, and in a layer applied to a sheet, the particles are in contact with each other to such an extent that good conductivity is obtained.

In Figs. 2 and 3, a building product is shown made with granular material as above prepared, the illustrations being necessarily somewhat diagrammatic. The base 10 of felt or other material is coated with the layer of plastic material 11, then the graded granular material is spread thereover and affixed by the application of pressure which causes a firm adherence or partial submergence of the grit. The metal deposit 13 is produced by ordinary electrolytic methods and it will be seen that the metal layer conforms to the irregular contour of the granular surface, each of the particles of which is a cathode surface on which metal collects. The granules include those of coarse size such as 14, and finer particles, such as 15 and 16, these finer particles lying between the coarse ones. The larger particles produce the major irregularities of the surface which afford means for securing the mechanical bond between base and metal, while the finer particles provide the contact between the larger particles so that the plating is continuous and may be made at a low current cost.

In some instances it may be desirable to avoid the careful grading and proportioning of the granular material to produce a mixture of the proper characteristics, and this can be done by having the material crushed to approximate maximum and minimum sizes, then embedding this material in the coating on the base and finally supplementing the contact between the adjacent particles by an application of fine conductive material, such as graphite or carbon flour. This should be done preferably while the asphaltic coating is hot so that any exposed parts of the coating will be covered by the graphite and act as an adhesive therefor.

The application of the graphite may be conveniently effected by sprinkling it on the sheet, then brushing or vibrating the sheet so that the graphite will settle into the interstices between adjacent granules, and then removing the excess. This last operation prevents the loose graphite from intervening between the plating and the embedded granules, thus detrimentally affecting the bond.

In Fig. 4 there is shown a building element

produced in accordance with the method just described. The base 10 has the coating layer 11 in which are embedded the granules of the conducting layer 12 over which is deposited the metal layer 13. It will be noted that the granules do not have the grading as to size and proportioning as to amount present in the case of the granules shown in Fig. 3, but the open spaces which would ordinarily occur between adjacent granules are now filled with graphite as at 17. In some instances, the graphite will contact with exposed portions of the base coating as at 18 while in others the powder will be wedged into the crevices between adjacent granules. In either case, the conductivity of the granular layer is greatly improved so that the metal may be deposited very readily in the form of a continuous sheet of substantially uniform thickness which is tightly bound to the base.

Fig. 5 is a plan view of a small portion of the surface ready for the plating operation, this surface being made of particles graded as to size and with the particles of different sizes proportioned as to amounts. It will be observed that the conductive layer consists of particles 19 of large size and finer particles, such as 20, which lie in the interstices between the particles 19. Such a conductive layer is made by proper grading of the particles and then proportioning the amounts of the particles of the different sizes so that although the final surface has an irregular contour, there is a substantially continuous contact between each particle and those which are adjacent to it. Furthermore, the area of such contacting surfaces throughout the sheet is quite large, owing to the use of the fine particles which lie in the interstices between the larger ones. This results in a layer of good electrical conductivity and there is thus produced a continuous layer of metal of substantially uniform thickness, and owing to the high conductivity of the cathode surface, the cost of plating current used in the plating operation is kept at a minimum.

The application of metal may be carried on by any convenient electrolytic process and may result in a plating over the entire surface of the base or over predetermined areas thereof only. For this latter purpose, the conductive material may be limited to those areas where metal is to appear, as at 21, the remainder 22 of the base being coated with a non-conductive material, or the entire base may be coated with conductive granular material and the deposit limited to selected areas by the use of a stencil or mask during the plating operation.

While I prefer to employ a non-metallic conductive granular material, such as coke, it is possible to secure good results with a metallic material such as granules or filings of copper, lead and other metals.

By employing the conductive grit graded

as to size and proportioned as to amount and with or without the graphite to secure an irregular conducting surface of the desired character, a superior product is secured. The presence of the fine particles of the grit between the larger particles, or the lodgment of the graphite between adjacent grit particles in the coating, tend to insure the production of a layer which is substantially continuous with respect to its conductivity and as the interstices are thus partially filled either with fine grit or graphite, as described, the depressions in the surface are partially filled, so that the depressions in the irregular surface are not so deep as would ordinarily occur. This has the effect of slightly smoothing out the irregular surface, but does not interfere with the obtaining of the mechanical bond. It does, however, result in securing a metal film which is of substantially uniform thickness, because it is found that in an ordinary granular layer the metal which enters the deep depressions between adjacent particles is not so thick as the metal which lies on the crests. This is because the crests lie closer to the anode in the plating cell and the metal has a natural tendency to collect on these crests for that reason. While the metal extends into the depressions, the metal film built up at these points is relatively thin. When the depressions are partially filled, either by grit particles of finer size or by graphite, the thickness of the metal layer throughout all portions of the coating tends toward substantial uniformity and furthermore, under these conditions, a better coverage is secured because there is less superficial area to be plated in the latter case than in the case of a layer in which the interstitial spaces are not partially filled. It is evident of course that these interstitial spaces must not be completely filled, as this would interfere with the strength of the mechanical bond, but it has been found possible to secure a satisfactory bond under the conditions I above suggest.

There is a further saving in the cost of production of the new material because a low percentage of imperfect elements is produced due to the superior conductivity of the cathode surface. Furthermore, there is also a saving of energy because in a surface in which the particles are not in contact it is possible, by continuing the plating operation, eventually to secure a film which is continuous throughout the base, but this requires that the metal plating should be built up so as to bridge the points not in contact, and in many instances this continuous film of metal can only be secured by carrying on the plating operation to a point such that the thickness of the film at some points on the base is much greater than is desired.

Owing to the fact that the new material includes the rough irregular surface on which

the metal is plated, the product is of attractive appearance because the metal coating is given a texture and the product is of long life, due to the complete protection afforded the base by the metal plating.

5 I claim:

1. A process for producing building elements suitable for roofing and similar purposes, which comprises crushing and grading electro-conductive granular material to produce a mixture containing selected amounts of particles of different sizes while substantially eliminating dust, applying a layer of such graded granular material to the surface of a base, said layer having high electrical conductivity and giving the base an irregular surface, applying a conductive powder thereover, the powder largely occupying the interstices between adjacent granules, and electro-depositing a layer of metal over the conductive surface so formed.

2. A building product suitable for roofing and other purposes, which comprises a base, a layer of material affixed to the surface of the base, this material being graded selected amounts of particles of different sizes, excluding dust to produce a layer in which each particle is in good electrical contact with the particles adjacent to it, certain of these particles being of a size sufficient to give the layer an irregular surface, and a coating of metal over the said layer and conforming to the irregularities thereof.

3. A process for producing building elements suitable for roofing and similar purposes which comprises affixing to the surface of a base a layer formed of a graded mixture of granules of electro-conductive material in which mixture all of the granules will pass through a screen of 14 mesh and a substantial proportion will be retained on a screen of 48 mesh, dust being substantially absent from the mixture, and electro-depositing a film of metal over the granular layer.

4. A process for producing building elements suitable for roofing and similar purposes, which comprises grading electro-conductive granular material to produce a mixture including a substantial proportion of granules of substantial size and a proportion of finer granules, particles of dust fineness being eliminated in the grading operation, affixing this mixture to the surface of a base to provide a layer of irregular surface contour due to the presence of the larger granules and of high electrical conductivity due to the finer granules lodged between and electrically connecting the larger granules, and electro-depositing a coating of metal over the granular layer.

60 In testimony whereof I affix my signature.  
RALPH E. DRAKE.